

# UNITED STATES PATENT OFFICE.

GEORGE W. LANGLEY, OF GREENBRIER, ARKANSAS, ASSIGNOR OF ONE-HALF TO NOAH T. S  
DEMPSEY, OF GREENBRIER, ARKANSAS.

## COMPOUND FOR TANNING HIDES.

No. 907,060.

Specification of Letters Patent.

Patented Dec. 15, 1908.

Application filed June 26, 1908. Serial No. 440,535.

*To all whom it may concern:*

Be it known that I, GEORGE W. LANGLEY, a citizen of the United States, residing at Greenbrier, in the county of Faulkner and 5 State of Arkansas, have invented new and useful Improvements in Compounds for Tanning Hides, of which the following is a specification.

This invention is an improved compound 10 for tanning hides and by means of which hides may be readily, quickly, and cheaply tanned into leather.

My improved compound consists of:

|    |                                                                       |             |
|----|-----------------------------------------------------------------------|-------------|
| 15 | Extract of buckeye or horse-chestnut ( <i>Æsculus hippocastanum</i> ) | 1 pound.    |
|    | Extract of poke-root ( <i>Phytolacca radix</i> )                      | 2 pounds.   |
| 20 | Gambier                                                               | 12 pounds.  |
|    | Water                                                                 | 20 gallons. |

I make the extract of buckeye or horse-chestnut by boiling 12 pounds of horse-chestnut bark in 6 gallons of water for about two 25 hours. I make the extract of poke-root by boiling 8 pounds of poke-root in 3 gallons of water for about 1½ hours.

Hides after they have been dehaired and scraped are placed in this improved tanning compound and kept therein for a suitable 30 length of time. Where the hide is light, it is usually necessary to keep the same in the compound from twenty four to forty eight hours. Upper leather requires ordinarily to be kept in the compound for from five to six 35 days. Heavy harness and sole leather requires usually from ten to fifteen days. The tanner by observing the color of the hide can judge when it has been sufficiently tanned.

Having thus described the invention, what 40 I claim is:—

A tanning compound consisting of extract of horse-chestnut, extract of poke-root, gambier and water, substantially in the proportions specified. 45

In testimony whereof I affix my signature in presence of two witnesses.

GEORGE W. LANGLEY.

Witnesses:

W. C. KELSO,  
D. GLOVER.